

## UNITED STATES PATENT OFFICE

PHILIP G. WRIGHTSMAN, OF CHESTER, PENNSYLVANIA, ASSIGNOR TO E. I. DU PONT  
DE NEMOURS & COMPANY, OF WILMINGTON, DELAWARE, A CORPORATION OF DELA-  
WARE

## NITRATED CARBOHYDRATE EXPLOSIVE AND PROCESS OF MANUFACTURE

No Drawing.

Application filed August 17, 1928. Serial No. 300,400.

This invention relates to a process of nitrating carbohydrates and polyhydroxy alcohols having from four to six carbon atoms by mixing them with liquid polyhydroxy alcohols and subjecting them to the action of a nitrating acid, and more particularly to the nitration of solutions of sucrose and sorbitol in either glycerin or glycol, and also to the explosive produced thereby.

10 Solutions of carbohydrates, such as sucrose and glucose in liquid polyhydroxy alcohols, such as glycerin and ethylene glycol, have been used in the manufacture of liquid dynamite ingredients. Considering yield, stability, explosive properties, etc., the most satisfactory carbohydrate has been sucrose in the form of cane or beet sugar. Its use in solution has been thus far practically limited to a maximum of 20% to 25%, owing to its solubility in and rate of crystallization out of polyhydric alcohol medium. Higher proportions of carbohydrates in solution may be employed by using more soluble carbohydrates, such as glucose or fructose, but these aldoses and ketoses are not as desirable as sucrose, principally because of low yield and instability.

15

20

25

This invention has as an object the development of a process for the nitration of solutions of carbohydrates and polyhydroxy alcohols having from four to six carbon atoms in liquid polyhydroxy alcohols. A further object is to produce a liquid explosive having a relatively high carbohydrate content, and having a substantially low freezing point. Further objects will appear hereinafter.

These objects are accomplished by the following invention which consists essentially in nitrating a mixture of carbohydrates and polyhydroxy alcohols having from four to six carbon atoms and liquid polyhydroxy alcohols.

The materials constituting the starting materials used in the process of my invention are carbohydrates, polyhydroxy alcohols having from four to six carbon atoms, and liquid polyhydroxy alcohols.

The carbohydrates may be either sucrose, 45 glucose, or fructose, or other carbohydrates,

but I prefer to use sucrose, although my invention is not limited to its use.

The polyhydroxy alcohols having from four to six carbon atoms which I have found satisfactory are those containing from four to six carbon atoms. It is not necessary that each carbon atom contain a hydroxyl group. For instance, I may use mannitol, sorbitol, dulcitol, ramnitol, arabitol, xylitol, pentaerythritol, erythritol, or other similar compounds which will be apparent from the disclosure herein. One method of preparing these compounds is by hydrogenating the desired aldoses or ketoses. It has been found that these hydrogenated sugars possess the advantages of good stability, high nitrogen, and excellent explosive properties. It is highly desirable to use nitrated polyhydroxy alcohols having from four to six carbon atoms in nitrated carbohydrate explosives, since it is more economical to use carbohydrate ingredients as freezing point depressants. One feature of my invention is the increase in the proportion of carbohydrate and the lowering of the freezing point of the explosive by using a mixture of carbohydrate and hydrogenated carbohydrate. The polyhydroxy alcohols having from four to six carbon atoms which I have found satisfactory need not be produced by the process of hydrogenation, however, but may be obtained from other sources, if desired.

I have also discovered that mixtures of nitrated carbohydrates and nitrated polyhydroxy alcohols having from four to six carbon atoms can be successfully employed with nitrated liquid polyhydroxy alcohols in the preparation of low freezing liquid explosives satisfactory for use in dynamites. I have further discovered that by dissolving a polyhydroxy alcohol having from four to six carbon atoms in addition to a carbohydrate in a liquid polyhydroxy alcohol medium, the practical maximum proportion of carbohydrate may be retained in solution in addition to substantial proportions of polyhydroxy alcohols having from four to six carbon atoms and that these solutions are satisfactory for use in the production of ex-

losive oils suitable for commercial explosive compositions.

The liquid polyhydroxy alcohols which I have found especially suited to the process of my invention are glycerin, diglycerin, and the glycols, such as ethylene glycol, for example. By increasing the proportion of glycol, the viscosity of the nitrated product is lowered, and as a consequence the resulting explosive contains high proportions of nitrated carbohydrates and nitrated polyhydroxy alcohols having from four to six carbon atoms, and is more easily handled in manufacture.

Although I may use any carbohydrate and any polyhydroxy alcohol having from four to six carbon atoms in any liquid polyhydroxy alcohol medium, a preferred example of my invention is a solution of 15% to 25% sucrose and from 5% to 50% sorbitol dissolved or suspended in the glycerin, or ethylene glycol, or a mixture of glycerin and ethylene glycol. Although it is not essential, I prefer to dissolve the carbohydrate and polyhydroxy alcohol having from four to six carbon atoms. But either or both may be suspended in the mixture, or the polyhydroxy alcohol having from four to six carbon atoms may be nitrated alone, before or after the other ingredients.

*Example.*—In carrying out my process, the proportions of carbohydrate, and polyhydroxy alcohols having from four to six carbon atoms and liquid polyhydroxy alcohols may, for example, be as follows:

|                            |
|----------------------------|
| 20% to 25% sucrose         |
| 10% to 40% sorbitol        |
| 10% to 60% glycerin        |
| 10% to 60% ethylene glycol |
| 15% to 25% sucrose         |
| 5% to 50% sorbitol         |
| 25% to 80% glycerin        |

It is, of course, to be understood that I may use any carbohydrate and any polyhydroxy alcohol having from four to six carbon atoms in any liquid polyhydroxy alcohol medium. Although it is not essential, it is desirable that the carbohydrate and polyhydroxy alcohol having from four to six carbon atoms be dissolved, but either or both may be suspended in the mixture or the polyhydroxy alcohol having from four to six carbon atoms may be nitrated alone, or before or after the other ingredients. The nitration, separation, washing, and neutralization are carried out in the same manner as is usually employed in the case of solutions of cane sugar in glycerin. A stabilizer such as diphenylamine may be added, if desired.

By proceeding in the manner I have described, I obtain an explosive having a relatively high proportion of carbohydrate, a

low freezing point, and a low viscosity. The explosive oil thus produced is an excellent explosive and may be handled with facility. As many apparently widely different embodiments of this invention may be made without departing from the spirit thereof, it is to be understood that I do not wish to limit myself to the specific embodiments thereof, except as indicated in the appended claims.

I claim:

1. The process of producing explosives which comprises nitrating mixtures of carbohydrates and polyhydroxy alcohols having from four to six carbon atoms and liquid polyhydroxy alcohols.

2. A process of producing explosives containing nitrated carbohydrate which comprises nitrating carbohydrates and polyhydroxy alcohols having from four to six carbon atoms in a liquid polyhydroxy alcohol medium.

3. A process of producing explosives containing nitrated carbohydrate comprising nitrating a solution of carbohydrate and polyhydroxy alcohol having from four to six carbon atoms in liquid polyhydroxy alcohol, said solution containing more than 5% polyhydroxy alcohol having from four to six carbon atoms and the practical maximum proportion of carbohydrate.

4. The process of producing liquid explosives containing nitrated carbohydrates which comprises nitrating a mixture of carbohydrates and polyhydroxy alcohols containing from four to six carbon atoms in liquid polyhydroxy alcohol medium.

5. The process of claim 4 wherein the carbohydrate is sucrose.

6. The process of claim 4 wherein the solid polyhydroxy alcohol having from four to six carbon atoms is taken from a group including erythritol and sorbitol.

7. The process of claim 4 wherein the liquid polyhydroxy alcohol is a mixture of glycerin and ethylene glycol.

8. The process of claim 4 wherein the liquid polyhydroxy alcohol is taken from a group consisting of ethylene glycol and glycerine.

9. A process of producing explosives comprising nitrating a mixture of sucrose, polyhydroxy alcohol taken from a group consisting of erythritol and sorbitol and a liquid polyhydroxy alcohol.

10. A process of producing explosives which comprises nitrating a mixture of sucrose, sorbitol, and a liquid polyhydroxy alcohol taken from a group consisting of glycerin and ethylene glycol.

11. A process of producing explosives which comprises nitrating a mixture containing from 15 per cent to 25 per cent of sucrose, 5 per cent to 50 per cent of sorbitol, and a liquid polyhydroxy alcohol.

12. An explosive comprising a nitrated carbohydrate, nitrated polyhydroxy alcohol having from four to six carbon atoms, and nitrated liquid polyhydroxy alcohol.
- 5 13. An explosive which comprises nitrated sucrose, nitrated polyhydroxy alcohol taken from a group consisting of erythritol and sorbitol, nitroglycerin and ethylene glycol dinitrate.
- 10 14. An explosive which comprises the nitrated mixture of 20% to 25% sucrose and 10% to 50% polyhydroxy alcohol taken from a group consisting of erythritol and sorbitol and the remainder polyhydroxy alcohol.
- 15 15. An explosive which comprises the nitrated mixture of 20% to 25% sucrose and 10% to 50% polyhydroxy alcohol taken from a group consisting of erythritol and sorbitol and the remainder a mixture of glycerin and ethylene glycol.
- 20 16. An explosive which comprises the nitrated mixture of 20% to 25% sucrose and 10% to 50% sorbitol and the remainder polyhydroxy alcohol taken from a group consisting of glycerin and ethylene glycol.

In testimony whereof, I affix my signature.  
PHILIP G. WRIGHTSMAN.

20

35

40

45

50

55

60

65